

# UNITED STATES PATENT OFFICE.

SAMUEL A. McCUNE, OF CENTERVILLE, IOWA.

## FORMULA FOR PAINT.

1,411,971.

Specification of Letters Patent. Patented Apr. 4, 1922.

No Drawing.

Application filed February 12, 1921. Serial No. 444,356.

To all whom it may concern:

Be it known that I, SAMUEL A. McCUNE, a citizen of the United States, residing at Centerville, in the county of Appanoose and 5 State of Iowa, have invented certain new and useful Improvements in a Formula for Paint, of which the following is a specification.

This invention relates to a mineral painting composition and has for its object the 10 production of a simple and efficient painting composition which is especially adapted for painting boiler heads, smoke stacks, steam and stand pipes, and in fact in all places and 15 under all conditions where it is absolutely necessary for the paint to be weather, heat and acid proof.

Another object of this invention is the 20 production of a simple and efficient painting composition which is adapted for use upon all materials subjected to atmospheric conditions.

The painting composition comprises the following ingredients:

25 1 gallon of coal tar, copperas in powdered form 12% of a pound, benzine  $\frac{1}{2}$  gallon or 12 $\frac{1}{2}$ %, litharge commercial 20% of 1 lb., plaster Paris 20% of 1 lb., rosin powdered 20% of 1 lb., sugar of lead 5% of 1 lb., 30 graphite powdered  $\frac{1}{2}$  pound, turpentine 1 $\frac{1}{4}$ % of 1 gal.

The painting composition above set forth will produce a very efficient mineral paint which is especially adapted for use in painting boiler heads, smoke stacks, steam and 35 stand pipes, metal bridge construction and all surfaces which are subjected to weather, heat and acid. The painting composition is of such a character as to prevent the scaling of the surface upon which the paint is 40 applied.

What is claimed is:

1. A painting composition comprising coal tar, copperas, benzine, commercial litharge, plaster of Paris, powdered rosin, 45 sugar of lead, powdered graphite and turpentine.

2. A painting composition comprising the following ingredients: coal tar one gallon, copperas in powdered form 12% of a pound, 50 benzine,  $\frac{1}{2}$  gallon or 12 $\frac{1}{2}$  of 1 lb., commercial litharge, 20% of 1 lb., plaster Paris 20% of 1 lb., powdered rosin, 20% of 1 lb., sugar of lead, 5% of 1 lb., graphite powdered  $\frac{1}{2}$  pound and turpentine, 1 $\frac{1}{4}$ % of 1 gal. 55

In testimony whereof I affix my signature in presence of two witnesses.

SAMUEL A. McCUNE.

Witnesses:

C. P. LILLMONT,  
J. A. SHANKS.